

## UNITED STATES PATENT OFFICE

EDWARD A. NILL, OF CLEVELAND, OHIO, ASSIGNOR TO THE PANOLEUM COMPANY, OF CLEVELAND, OHIO, A CORPORATION OF OHIO

ABRASIVE COMPOSITION

No Drawing.

Application filed October 18, 1927. Serial No. 227,058.

This invention relates to an abrasive composition and the method of compounding the same by which the properties of the composition may be varied to adapt the same to 5 different uses, the invention being particularly applicable to abrasive compositions suitable for application to a buffing wheel.

The present invention has for an object to provide an abrasive composition in the form 10 of a solid substance of smooth and homogeneous consistency which has a relatively high percentage of finely divided abrasive material uniformly incorporated therein and which can be readily molded into the desired form.

15 A further object of the invention is to provide a solid abrasive composition in which the binder is of relatively low melting point and in its liquid state of relatively high viscosity so that, when a stick of the abrasive composition 20 is applied to the surface of a rapidly rotating buffing wheel, the portion of the stick in contact with the wheel is softened by the heat generated by the friction and adheres to the surface of the wheel without loss of abrasive material due to crumbling or breaking off of particles of the stick.

25 A further object is to provide a composition which after being applied to a buffing wheel will not stick to the metal being polished in the buffing operation.

30 A further object is to provide an abrasive composition and a method of making the same by which the melting point and consistency may be regulated by varying the 35 proportions of the constituents to produce compositions which possess the consistency and melting point found to be most desirable for buffing wheels operating at different speeds and on different kinds of material.

40 A further object is to provide an abrasive composition in which the binder in its liquid state is of such high viscosity that even when subjected to relatively high temperatures in the operation of a buffing wheel, the binder 45 will retain the abrasive on the wheel.

45 A further object is to provide a binder which after the abrasive material is mixed therewith solidifies very quickly preventing any appreciable settling of the heavier abrasive materials.

With the above and other objects in view the invention may be said to comprise the composition and method of compounding the same as hereinafter described and particularly set forth in the appended claims, together with such variations and modifications thereof as will be apparent to one skilled in the art to which the invention appertains.

55 The present invention utilizes a property which has been found to be possessed to a high degree by anilids of fatty acids when mixed with mineral oils, fatty oils and waxes, namely, the property of stiffening the consistency of the mixture or solution to an extent varying with the percentage of anilid employed. The anilid also possesses the 60 property of raising the solidifying point which is advantageous in a composition of this character.

65 In making the binder, a relatively large percentage of mineral oil is mixed with a relatively small percentage of a fatty oil, together with the percentage of anilid, preferably stearanilid, necessary to give the composition the desired consistency. By employing mineral oils of different viscosities and by varying the relative proportions of mineral and fatty oils as well as the proportion of anilid, compositions may be obtained 70 of any desired consistency and solidifying point within relatively wider limits than is 75 customarily obtainable.

80 In making the abrasive blocks or sticks, a finely divided abrasive such as emery, carbondum, silica, tripoli, whiting, lime, rouge, crocus, chrome or any combination of these abrasive substances is intimately mixed with the binder after which the blocks or sticks are molded to the desired form. The 85 percentage of the abrasive in the composition will vary somewhat with the character of the abrasive material and the use to which the abrasive is to be put, but an important advantage of the binder of the present invention is that it is capable of retaining a very 90 large percentage of abrasive material uniformly dispersed throughout the body thereof without becoming brittle and unworkable.

95 While it is to be understood that the proportions of the ingredients may be varied to 100

quite an extent to obtain compositions suitable for different kinds of work, a typical composition may be made as follows:

5 Finely divided abrasive, 65% to 75%, binder, 25% to 35%, in which the binder is composed of the following ingredients, stearanilid 30%, petrolatum 55%, tallow 15%. The composition above described will have a melting point of approximately 157° F. and 10 normally is substantially of cup grease consistency.

It will be understood that by increasing the proportion of stearanilid, the consistency will be increased and the solidifying point 15 will be raised and that by employing mineral oils of different viscosities and different proportions of fatty oil, any desired consistency and solidifying point within a relatively wide range may be obtained. If stiffer 20 consistency is desired, the percentage of petrolatum and tallow may be reduced or either or both of these ingredients may be omitted altogether and stearanilid used alone as a binder. The petrolatum may be of an inexpensive 25 quality, other anilids of fatty acids may be substituted for the stearanilid, and the tallow which is added to increase the lubricating and clinging quantities may be replaced by other waxes such as stearic acid, 30 or paraffine wax or by fatty oils such as commercial oleic acid, cotton seed oil, fatty acid, or corn oil fatty acid.

An abrasive stick formed of composition of the present invention when applied to a 35 rapidly rotating surface of a buffering wheel gradually softens at the end due to the heat generated by frictional engagement with the wheel and the combustion as it is melted by the heat is gradually and uniformly distributed over the surface of the wheel. Furthermore, due to the stiff consistency of the composition and the uniform distribution of the abrasive materials therein, the abrasive material is firmly held on the buffering wheel during 40 polishing operations even though relatively high temperatures are produced by the frictional engagement of the wheel with the article being polished. In addition, clean bright surfaces are produced in the buffering 45 operation due to the fact that the binder possesses high lubricating qualities and adheres firmly and uniformly to the buffering wheel and does not cling to the surface of the metal being polished.

50 55 What I claim is:

1. An abrasive stick composed of a suitable finely divided abrasive and a homogeneous wax-like substantially anhydrous binder composed of mineral and fatty oils having a 60 substantial proportion of stearanilid in solution therein.

2. An abrasive stick composed of a suitable finely divided abrasive incorporated in a homogeneous wax-like substantially anhydrous binder composed of mineral oil 40 to 60%,

a fatty oil 10 to 20% and stearanilid 20 to 40%.

3. An abrasive stick composed of a suitable finely divided abrasive incorporated in a homogeneous wax-like substantially anhydrous 70 binder composed of petrolatum 55%, stearanilid 30%, and tallow 15%.

4. An abrasive stick composed of a homogeneous wax-like substantially anhydrous binder composed of mineral and fatty oils 75 having a substantial proportion of an anilid of a fatty acid in solution therein, and particles of abrasive material uniformly interspersed throughout the binder.

In testimony whereof I affix my signature. 80  
EDWARD A. NILL.

85

90

95

100

105

110

115

120

125